

T. H. MATHIAS.

METHOD OF ROLLING DEEP FLANGED SHAPES.  
APPLICATION FILED MAY 28, 1912.

1,082,756.

Patented Dec. 30, 1913.

2 SHEETS—SHEET 1.

Fig. 1.

NEW PROCESS



Fig. 4.

Fig. 3.



Fig. 5.



WITNESSES.

J. M. Millward  
Allan H. Gross

INVENTOR  
Thomas H. Mathias  
BY  
Alfred Wilkinson  
ATTORNEY

T. H. MATHIAS.  
METHOD OF ROLLING DEEP FLANGED SHAPES.  
APPLICATION FILED MAY 28, 1912.  
1,082,756.

Patented Dec. 30, 1913.

2 SHEETS—SHEET 2.

OLD PROCESS



Fig. 6.



Witnesses:  
M. Millward  
Allan T. Foss.

Inventor  
Thomas H. Mathias  
By his Attorney  
Alfred Wilkerson

# UNITED STATES PATENT OFFICE.

THOMAS H. MATHIAS, OF BUFFALO, NEW YORK, ASSIGNOR TO LACKAWANNA STEEL COMPANY, OF LACKAWANNA, NEW YORK, A CORPORATION OF NEW YORK.

## METHOD OF ROLLING DEEP-FLANGED SHAPES.

1,082,756.

Specification of Letters Patent.

Patented Dec. 30, 1913.

Application filed May 28, 1912. Serial No. 700,189.

*To all whom it may concern:*

Be it known that I, THOMAS H. MATHIAS, a citizen of the United States, residing at Buffalo, in the county of Erie and State of New York, have invented new and useful Improvements in Methods of Rolling Deep-Flanged Shapes, of which the following is a specification.

My invention relates to the rolling of structural steel shapes or sections, and consists in a new process of rolling involving a new principle, whereby absolutely new forms of beams may be produced, that is beams of substantial size for structural purposes having integral, middle or intermediate flanges of substantial length. The new principle, which I have discovered, is that the flanges can be formed and worked down in closed passes, whereas it has heretofore been believed that this could only be done in open passes. My process involves said principle applied as described. The rolls of each and every pass and on one or both sides are provided, adjacent the middle of the roll, with the closed grooves to form these middle flanges. The closed grooves of the successive passes are so proportioned to each other that at every pass the middle flange about to enter the closed groove is substantially thicker than said groove and a substantial draft is applied to the flange in said groove, but the surplus for the closed groove is throughout the entire process always less than the surplus on the end flanges for the open grooves.

Fully to explain my invention, it is necessary to understand the established practice in rolling structural sections provided with edge flanges such as I beams and channels. The forming and working down of these flanges is all done in open grooves, and each closed groove is of sufficient width merely to receive the flange which has been worked down in the immediately preceding open groove. In other words, the flange, as it leaves each open groove is worked down to such a thickness, as to be free to enter the next closed groove (though of course it must fit the closed groove snugly) and therefore pass through such closed groove with practically no draft applied to it. The edge flanges are worked down exactly as is the web, that is when between, and only when between, the opposed surfaces of the two rolls, that is in open grooves; where flanges are formed on both sides of the section as in I beams,

it is evident that in only half of the grooves will the flange be between the said opposing surfaces, that is, in the open grooves; the bar will then be reversed so that in the other half of the grooves the flange will lie dead and unworked in the closed grooves while the reduction is being continued on the web and the opposite flanges. For it has always been believed that no substantial reduction could be effected in rolling except between opposed rolls, and that the work of rolling down the flanges, just as the web, must be effected between the opposed surfaces of two rolls, that is in the open groove. The whole system of rolling flanged sections, and the design and construction of the rolls, have been based on this belief and practice. As a radical departure from this practice I have discovered, what has never before been considered possible, that is the principle that flanges may be worked down in closed grooves and I have embodied this principle in my new process. To practise that process, the rolls must be properly formed with closed grooves at or about their middle, and on one, or both, rolls at each pass, according as the middle flange is to be formed on one, or both, sides of the web of the section. And these closed grooves in the successive passes must be proportioned one to the other so that the flange is substantially thicker than the closed groove into which it enters at every pass. The bar is first roughly shaped in the blooming mill with the middle flange substantially wider than the middle groove of the first roughing and finishing rolls. When the shape is put through the first of these rolls, a substantial draft is applied to the middle flange, whether such a flange is to be produced on one or both sides of the web, and said flange is substantially worked down in said first pass. This same proportion of the flange and this same application of a substantial draft thereto must be maintained at every successive pass, but, as aforesaid, there is always maintained a substantially less surplus on the middle flange for each and every closed groove, than on the end flanges for the open grooves. Furthermore there must be some surplus of metal in the web, and the web must be made thin at the beginning. The thinner the web in the cogging mill, the more certainty of filling the central flange because there is less draft on the web (and here there is more to

be done on the section as a whole). Therefore I roll down the web in the cogging mill as thin as reasonably possible, and yet no matter how thin, there must still be left 5 in the web, all through the rolling, some surplus to insure the flange. To that end I pass the shape through the blooming mill more times than in the usual processes, say about thirty times, more or less, as compared 10 to about twenty, more or less, so that the web will be comparatively thin when the section comes to the first of the roughing rolls and thereafter there will be less reduction on the web at each pass.

15 For the sake of illustration I have shown my invention applied to producing an I beam with middle flanges, but it may be applied to rolling other shapes with a middle flange, or flanges. Heretofore when shapes 20 with substantial intermediate flanges were required, it was necessary to form the shapes for the flanges separately and then secure them to the web of the beam in any suitable way as by riveting.

25 In the drawing herewith, the reference letters and numerals of this description indicate the corresponding parts in all the figures.

Figure 1 is an elevation of a portion of a 30 train of rolls, in which four passes are shown with the grooves so shaped and proportioned as to roll by my process an I beam with middle flanges on both sides. Fig. 2 is a similar elevation showing the production of the usual form according to 35 the established practice which has been followed for many years. Fig. 3 is a diagram showing substantially the comparative sizes of the ten (more or less) closed passes in the so called "roughing" 40 and "finishing" rolls, whereby the middle flanges are produced under my process. Figs. 4 and 5 show shapes which can be made by my process, and only by my process, as I believe. Figs. 6 and 7 show the 45 waste ends respectively of the usual I beam, and of the beam of my Figs. 1 and 3, to illustrate the difference in operation and the different factors involved in my process.

50 In both Figs. 1 and 2 I have shown, for forming I beam sections, four passes which will be sufficient to illustrate my invention but it will be understood that the bar will be put through at least about ten passes, 55 in which is done the roughing and the finishing, and that, as a preliminary step, the bloom is put through the blooming mill as aforesaid to form the shaped blank. In case of each groove the outline of the rolls 60 is in full lines, and the shape, about to be put through, in dotted lines. The flanges shown with the sharp corner (that is the edge flanges) have been worked down in the preceding open groove and are about to 65 enter the closed groove, where they are held

unreduced while the opposite flange is being worked down.

Referring first to Fig. 2, A', B', C', and D' indicate four passes, corresponding respectively to about passes 6, 7, 8 and 9 of the roughing and finishing rolls, of which commonly there will not be less than ten, though it is not necessary to show more than four to explain my invention.

At pass A' is indicated in dotted lines 75 the shape received from the preceding groove. On this shape the flanges 1 1, with the square corners, were reduced in the preceding open grooves and are now about to enter the closed grooves 2 on the top roll X. 80 These flanges are no thicker than these closed grooves, in some cases they are even thinner, so that they pass through these grooves without side draft or being reduced, while the flanges 3 from the preceding closed 85 grooves are being rolled down in the open grooves 4 between the collar on the top roll and the tongue of the middle roll Y. For that reason the groove 4 is made thinner than the flange 3. 5 indicates the web. 90

In pass B' the top flanges 1 1 are between the middle roll Y and the bottom roll Z (or the open groove) while the bottom flanges 3 are in the closed grooves 8. These closed 95 grooves 8 are of a width sufficient merely to receive freely the flanges 3, which had been rolled down in pass 4, and hold them, while flanges 1, from closed grooves 2, are rolled down in open groove 6, between the opposed surfaces of the two rolls. 100

In passes C' and D' the operation is the same; flanges 1 next going freely into the closed grooves 9 and being further rolled down in the open groove 10, while flanges 3 are rolled down in open groove 11, and 105 then drop freely into closed grooves 12.

In case of each closed groove there is shown a little surplus of metal on the extreme edge of the flange as indicated; this is merely to insure the filling out of the 110 edges, so that they shall be true, sharp and perfect and not for securing draft on the flanges; if there were no such surplus, the reduction on the web would have a tendency, due to elongation, to shorten the 115 flanges.

Referring now to Fig. 1, in which my process is shown applied to the production of a rolled I beam section having opposite middle flanges 20, A, B, C and D indicate 120 four passes corresponding (as do the four in Fig. 2) respectively to about passes Nos. 4 to 7 of the roughing and finishing rolls. I have provided in every groove, of which these four are illustrations, the opposite 125 closed grooves indicated by 21 in pass A. The flanges 20 are substantially wider than these closed grooves so as to have an ample surplus of metal on each side whereby there is a substantial side draft applied to these 130

figures as the bar goes through the rolls and the flanges are thus worked down. There is of course a progressively less total amount of reduction in each succeeding pass in which the center closed grooves are indicated respectively by 21 to 26 inclusive, but in each case it will be seen that the middle flange is substantially thicker than the closed groove, and this is an essential feature of my process, for reasons above given. The side flanges of this special I beam section on Figs. 1 and 4 are indicated by the same numerals as in Fig. 2 and they are produced by the process there indicated, for it is not necessary or desirable to vary that process on the side flanges. The grooves and passes of Fig. 1 for the edge flanges have the same reference numerals as in Fig. 2.

In Fig. 6 is shown the shape of the usual waste end of a rolled I beam section, in which the draft on the web, constantly tending to draw from the flanges rolled in the open grooves, has forced the web out into a sort of a rounded point.

Evidence of the new principles involved in my process is found in Fig. 7 showing the form of waste end in beams with middle flanges according to my process. Here the fish-tail form shows that the web does not draw from the flanges but the flanges from the web even though the web is rolled by the periphery of the roll where the speed is greatest, and shows the novelty and desirability of at least one of the steps of my process, that is, the initial thinning of the web.

In Figs. 4 and 5 I have shown an I beam and a sheet piling section, both provided with reinforcing middle flanges on both sides, whereby they are greatly strengthened. I believe that I am the first to have produced these shapes and that they can only be produced commercially by my process. The flanges on the pile section are also important in concrete protected piling for they may be punched or otherwise used to support the rods, wires or other elements for binding the concrete. While the middle flanges in various modifications of these shapes are produced by my process it will be understood that the rolls must be variously formed to produce these various shapes, and also to roll the variations in the edges of the beam, for instance in Figs. 4 and 5 are shown shapes in which edge flanges are present but very different in shape. The middle flanges may be rolled decidedly deeper than the edge flanges.

It will be understood that in all cases the middle flange is of substantial depth, for instance two or three inches or more, which must be produced by my process, as distinguished from a mere shallow rib, which may be merely forced out, without any proportioning of the parts, due merely to the

natural flow of the metal, in contrast to the abnormal flow produced in my process. I am aware that small shapes, such as bars for tie-plates have been rolled, provided with such short, intermediate ribs or flanges, but these are not true flanges, merely ribs or corrugations, which are not rolled or worked out but are merely forced out as aforesaid. It will be understood that for these tie-plates, an unshaped bar, substantially rectangular in cross-section, is put through the rolls three or four times and these ribs of perhaps  $\frac{1}{2}$ " to  $\frac{3}{4}$ " in length are forced out, without any special provision of metal therefor. They are forced out and can be forced out only to the extent permitted by the natural flow of the metal, there is no proportioning of the various parts of the bar one to the other, no proportioning of the middle flanges in the various passes to the respective closed grooves, no calculation of the particular amount of metal which must be provided, and no provision for the particular amount of metal, to fill those closed grooves. Whereas the clear distinction of my sections therefrom is that middle flanges can be produced of a length far beyond the natural or normal flow of the metal. The closed grooves are of such a depth that they can be filled only by my process. No amount of mere forcing would make the metal flow sufficiently to fill the groove, even if the rolls were strong enough to stand up to the work.

Having described my invention, I claim,

1. The process of rolling structural metal beams having a web and an intermediate flange of substantial depth, which consists in applying draft to said flange in each and every one of a series of closed grooves, the grooves in the successive passes being so proportioned that the flange will always be thicker than the width of the groove which the flange is entering, whereby said flange will be worked down gradually in a plurality of passes, but worked down to a certain extent in every pass.

2. The herein described process of rolling metal beams having edge flanges and intermediate flanges of substantial depth, which consists in applying draft to the intermediate flanges and reducing the same at each and every pass in closed grooves, but applying draft to the edge flanges and rolling down the same only in the alternate passes and then only in open grooves, and in the other alternate passes holding the edge flanges unreduced in closed grooves.

3. The process of rolling metal beams having edge flanges and intermediate flanges of substantial depth, which consists in reducing the edge flanges only in open grooves and the intermediate flanges only in closed grooves, the closed groove of the successive passes being so proportioned that the in-

termediate flange will always be thicker than the groove it is entering and be rolled down at each and every pass, but the edge flanges being rolled only in open grooves 5 between the surfaces of opposing rolls.

4. The process of rolling a metal beam having a web and an intermediate flange of substantial depth, which consists in reducing the beam successively in series of 10 passes, one of the rolls of each of said passes having a closed groove for said flange, of less width than the thickness of the flange as it enters said pass, said groove thus acting to reduce and to produce a draft 15 on said flange at each and every pass, but the successive grooves being so proportioned that there is gradually less reduction on the flange in each succeeding pass.

5. The process of rolling metal beams 20 having edge flanges and intermediate flanges of substantial depth, which consists in reducing the intermediate flanges in each and every pass in a closed groove, and reducing the edge flanges in alternate passes in open 25 grooves, the edge flanges being held unreduced in the other alternate passes in closed

grooves, the reduction of the edge flanges being greater in the passes in which they are being reduced than is the reduction of the intermediate flanges in the same passes. 30

6. The process of rolling a metal beam having a web and an intermediate flange of substantial depth, which consists in roughing the billet in the blooming mill so as to produce a shape with a thin web, then continuing the reducing of the beam successively in a series of passes, one of the rolls of each pass having a closed groove for the flange of less width than the thickness of the flange as it enters said pass, the 40 flange being reduced at each pass, the web being rolled down gradually between the opposing surfaces of the two rolls but being so proportioned that it has a surplus metal and is reduced at each pass. 45

In testimony whereof I have signed my name to this specification in the presence of two subscribing witnesses.

THOMAS H. MATHIAS.

Witnesses:

ASA C. BYAM,

WALTER J. BRYAN.